



US006033278A

# United States Patent [19]

Watkins et al.

[11] Patent Number: 6,033,278

[45] Date of Patent: Mar. 7, 2000

## [54] FIELD EMISSION DISPLAY WITH NON-EVAPORABLE GETTER MATERIAL

[75] Inventors: Charles M. Watkins; David A. Cathey, both of Boise, Iowa

[73] Assignee: Micron Technology, Inc., Boise, Id.

[21] Appl. No.: 09/127,014

[22] Filed: Jul. 31, 1998

## Related U.S. Application Data

[62] Division of application No. 08/755,589, Nov. 25, 1996, Pat. No. 5,789,859.

[51] Int. Cl. 7 ..... H01J 9/38

[52] U.S. Cl. ..... 445/41

[58] Field of Search ..... 445/41; 417/48; 417/51

## [56] References Cited

## U.S. PATENT DOCUMENTS

- |           |         |                 |       |         |
|-----------|---------|-----------------|-------|---------|
| 5,223,766 | 6/1993  | Nakayama et al. | ..... | 313/495 |
| 5,520,563 | 5/1996  | Wallace et al.  | ..... | 445/41  |
| 5,614,785 | 3/1997  | Wallace et al.  | ..... | 315/496 |
| 5,656,889 | 8/1997  | Niiyama et al.  | ..... | 313/553 |
| 5,688,708 | 11/1997 | Kato et al.     | ..... | 445/41  |

## OTHER PUBLICATIONS

E. Giorgi and B. Ferrario, High-Porosity Thick-Film Getters, IEEE Transactions on Electronic Devices, vol. 38, pp. 2744-2747 (Nov. 1989).

Primary Examiner—Kenneth J. Ramsey  
Attorney, Agent, or Firm—Dorsey & Whitney LLP

## [57] ABSTRACT

The present invention provides an FED with a getter material deposited and activated on the substrates of the faceplate and the baseplate of the FED. In one embodiment of the invention, a large FED includes a faceplate, a baseplate, and an unactivated non-evaporable getter material. The faceplate has a transparent substrate with an inner surface, and a cathodoluminescent material disposed on a portion of the inner surface. The baseplate has a base substrate with a first surface and an emitter array formed on the first surface. The baseplate and the faceplate are coupled together to form a sealed vacuum space in which the inner surface and the first surface are juxtaposed to one another in a spaced-apart relationship across a vacuum gap. The unactivated non-evaporating getter material is deposited directly on the inner surface and/or the first surface. The unactivated non-evaporating getter material may alternatively be deposited on a thin film of bonding material that is disposed on the inner surface and/or the first surface.

## 39 Claims, 4 Drawing Sheets





Fig. 1



Fig. 2 (Prior Art)



Fig. 3



Fig. 4 (Prior Art)

## FIELD EMISSION DISPLAY WITH NON-EVAPORABLE GETTER MATERIAL

### CROSS-REFERENCE TO RELATED APPLICATION

This application is a divisional of U.S. patent application Ser. No. 08/755,589, filed Nov. 25, 1996, and issued as U.S. Pat. No. 5,789,859.

This invention was made with Government support under Contract No. DABT63-93-C-0025 awarded by Advanced Research Projects Agency (ARPA). The Government has certain rights in this invention.

### TECHNICAL FIELD

The present invention relates to the use of getter materials in field emission displays, and, more particularly, to incorporating a non-evaporable getter material into an FED in a minimal amount of space.

### BACKGROUND OF THE INVENTION

Field emission displays (FEDs) are packaged vacuum microelectronic devices that are used in connection with computers, television sets, camcorder viewfinders, and other electronic devices requiring flat panel displays. FEDs have a baseplate and a faceplate juxtaposed to one another across a narrow vacuum gap. In large FEDs, a number of spacers are positioned between the baseplate and the faceplate to prevent atmospheric pressure from collapsing the plates together. The baseplate typically has a base substrate upon which a number of sharp, cone-shaped emitters are formed, an insulator layer positioned on the substrate having apertures through which the emitters extend, and an extraction grid formed on the insulator layer around the apertures. Some FEDs, and especially smaller FEDs, also have a backplate coupled to the faceplate such that the backplate encloses the baseplate in a vacuum space. The faceplate has a substantially transparent substrate, a transparent conductive layer disposed on the transparent substrate, and a photoluminescent material deposited on the transparent conductive layer. In operation, a potential is established across the extraction grid and the emitter tips to extricate electrons from the emitter tips. The electrons pass through the holes in the insulator layer and the extraction grid, and impinge upon the photoluminescent material in a desired pattern.

One problem with FEDs is that the internal components continuously outgas, which causes the performance of FEDs to degrade over time. The effects of outgassing are minimized by placing a gas-absorbing material (commonly called getter material) within the sealed vacuum space. Accordingly, to absorb the gas in the vacuum chamber over an FED's lifetime, a sufficient amount of getter material must be incorporated into the FED before it is sealed. Also, a sufficient amount of space must be allowed between the getter material and the component parts of the FED to allow a passageway for the gas to travel to the surface area of the getter material.

In conventional FEDs, the getter material is deposited and activated on a metal plate separately from the other component parts of the FED. Getter material is activated by heating it to a temperature at which a passivation layer on its exposed surfaces is diffused. Non-evaporable getter materials used in FEDs activate at approximately 900° C. The base substrate, transparent substrate and backplate, however, are generally made from materials that begin to deform at approximately 450° C.-500° C., the temperature range at

which many glass substrates and semiconductor substrates anneal. Accordingly, in order to avoid damaging the substrates, unactivated getter material is conventionally deposited and then activated on a metal plate apart from the substrates. The metal plate with activated getter material is then mounted on one of the substrates of an FED. The metal plate and getter material together are generally about 150  $\mu\text{m}$  thick.

The metal plate and getter material are mounted on small FEDs differently than they are on large FEDs. In small FEDs, the metal plate is generally mounted on a support member between the backplate and the baseplate. In large FEDs, the metal plate is commonly mounted on either the faceplate, the baseplate, or in a pump out tube.

Conventional FEDs and manufacturing methods present unique problems for incorporating getter material into the display assemblies because the distance between the faceplate and baseplate should be minimized. One problem is that the thickness of the metal plate and getter material together is a limiting factor in reducing the distance between the faceplate and the baseplate. In large FEDs, the distance between the faceplate and the baseplate is desirably 25  $\mu\text{m}$ -200  $\mu\text{m}$ ; the 150  $\mu\text{m}$  thickness of the getter material and metal plate, therefore, often requires the faceplate and baseplate to be spaced apart by more than the desired distance. Another problem is that the metal plate increases the cost to manufacture an FED because it is a separate part and must be securely attached to another component part of the FED to prevent it from coming loose. Loose metal plates are a significant problem in FEDs because small particles of getter material may break away from a loose plate, causing shorting to occur across the emitter tips.

In light of the problems associated with incorporating getter material on a metal plate into conventional FEDs, it would be desirable to develop an FED and a method of manufacturing an FED in which non-evaporable getter materials are securely attached to the FED in a minimal amount of space and are activated after being incorporated in the FED.

### SUMMARY OF THE INVENTION

The present invention is an inventive FED with a getter material that is deposited and activated on the substrates of the faceplate, baseplate and/or backplate. In one embodiment of the invention, a large FED includes a faceplate, a baseplate, and an unactivated non-evaporable getter material. The faceplate has a transparent substrate with an inner surface and a cathodoluminescent material disposed on a portion of the inner surface. The baseplate has a base substrate with a first surface and an emitter array formed on the first surface. The baseplate is coupled to the faceplate so that the inner surface and the first surface are juxtaposed to one another in a spaced-apart relationship across a vacuum gap. The unactivated non-evaporating getter material for absorbing gas within the space is deposited directly onto the inner surface and/or the first surface.

In another embodiment of the invention, a small FED includes a faceplate, a backplate, a baseplate, and an unactivated non-evaporable getter material. The faceplate has a transparent substrate with an inner surface and a cathodoluminescent material disposed on the inner surface. The backplate has an interior surface coupled to the faceplate so that the interior surface and the inner surface form a sealed chamber in which a vacuum is drawn. The baseplate has a base substrate with a first surface, a second surface, and an emitter array formed on the first surface. The baseplate is

coupled to the faceplate such that the inner surface and the first surface are juxtaposed to one another in a spaced-apart relationship in the vacuum chamber. The unactivated non-evaporating getter material for absorbing outgassed matter within the vacuum gap is deposited directly onto the inner surface, the interior surface, the first surface, and/or the second surface.

In an embodiment of the method of the invention, an unactivated getter material is deposited on a surface of a substrate that is a component part of either the faceplate or the baseplate. The getter material is then selectively heated to its activation temperature by a focused energy source while it is on the substrate.

#### BRIEF DESCRIPTION OF THE DRAWINGS

FIG. 1 is a cross-sectional view of a portion of a large field emission display with a getter material incorporated therein in accordance with the invention.

FIG. 2 is a cross-sectional view of a portion of a conventional large field emission display with a getter material.

FIG. 3 is a cross-sectional view of a small field emission display with a getter material incorporated therein in accordance with the invention.

FIG. 4 is a cross-sectional view of a conventional small field emission display having a getter material.

#### DETAILED DESCRIPTION OF THE INVENTION

FIGS. 1 and 3 illustrate the inventive FEDs of the present invention in which an unactivated getter material is deposited and then subsequently activated on the substrates of the faceplate, baseplate and/or backplate. The present invention solves the problems associated with incorporating getter material into conventional FEDs by eliminating the metal substrate upon which getter material is conventionally deposited and activated; instead, the present invention deposits unactivated, non-evaporable getter material onto the substrates of the faceplate, baseplate, or backplate. An important aspect of the present invention is that the getter material is activated after it has been deposited on the substrates by selectively heating the getter material to its activation temperature of approximately 900° C. without heating the substrates above their annealing temperatures of approximately 450–500° C. for any significant period of time. Specific features of the invention and its advantages are described in detail herein.

FIG. 1 illustrates a portion of a large FED with a faceplate 10, a baseplate 50, and a vacuum gap 40 therebetween in which a vacuum is drawn. The faceplate 10 has a transparent substrate 15 with an inner surface 11 facing the vacuum gap 40 and an outer surface 12 exposed to the atmosphere. The transparent substrate 15 is generally made from glass that begins to deform at approximately 450–500° C. An electrically conductive layer of material 20 and a cathodoluminescent layer of material 22 are disposed on the inner surface 11 across a portion of the transparent substrate 15. The baseplate 50 has a base substrate 55 with a first surface 51 that faces the inner surface 11 of the faceplate 10 and a second surface 52 that defines the backside of the baseplate 50. The base substrate 55 is preferably made from a type of glass that also anneals at approximately 450–500° C. A second layer of conductive material 53 is disposed on the first surface 51 of the base substrate 55, and a large number of emitters 54 are formed on the conductive material 53. A dielectric material 56 is positioned on the conductive mate-

rial 53 and the base substrate 50, and a number of holes are etched in the dielectric material 56 around and above the emitter tips 54. An extractor grid 58 is positioned on top of the dielectric material 56. The extractor grid 58 has a number of openings 59 positioned over the tips of the emitters 54 to allow electrons to pass through the grid 58 to the cathodoluminescent material 22. The faceplate 10 and baseplate 50 are maintained in a spaced-apart relationship under the influence of the vacuum by a number of spacers 30 positioned at various locations throughout the FED.

A getter material 90 is deposited in its unactivated state on the inner surface 11 of the faceplate 10 and/or the first surface 51 of the baseplate 50. The getter material 90 is a non-evaporable getter material that is preferably made from a titanium and zirconium alloy. Two suitable non-evaporable getter materials are a titanium and Zr84-A116 alloy, and a titanium and Zr70-V24.6-Fe5.4 alloy manufactured by SAES Getters, SpA. Other suitable non-evaporable getter materials include molybdenum and thorium. The getter material 90 may be deposited directly on the substrates by electroplating, screen printing, settling out of solution, electrophoresis processing, or other suitable deposition processes. In another embodiment, the getter material 90 may be deposited on the sides of the spacers 30 to increase the amount of getter material in the large FED 100. The thickness of the getter material 90 depends upon the amount of getter material that is required for a specific design and the total surface area within the FED 100 upon which the getter material 90 may be deposited. The getter material 90 is generally between 10  $\mu\text{m}$  and 100  $\mu\text{m}$  thick.

In a preferred embodiment, a thin film of bonding material 92 is disposed onto the surface of the substrate 55 of the baseplate 50 before the getter material 90 is deposited onto the substrate 55. The bonding material 92 may also be disposed onto the faceplate substrate 15. The bonding material 92 is preferably a very thin layer of nickel that is approximately 1–20  $\mu\text{m}$  thick. Other suitable bonding materials include nickel-chrome, stainless steel, molybdenum, titanium and zirconium. The bonding material 92 provides a stronger bond between the getter material 90 and the substrates 15 and 55. Accordingly, the bonding material 92 reduces the risk that a particle of getter material 90 will break away from the substrates 15 or 55.

After the getter material 90 has been deposited onto the faceplate 10, baseplate 50, and/or spacers 30, it must be activated in a vacuum without deforming or otherwise ruining the substrates 15 and 55. As discussed above, a non-evaporable getter material is activated by heating it to approximately 900° C. to cause a passivation layer on its exposed surfaces to diffuse. Because the annealing temperature of the substrates 15 and 55 is only about 450–500° C., one important aspect of the invention is the process by which the getter material 90 is activated at 900° C. after it has been deposited on the substrates 15 or 55 without deforming or otherwise damaging the substrates.

The getter material 90 is activated while on the substrates 15 and 55 by selectively heating the getter material 90 with a focused, high-intensity energy source 95 such as a microwave emitter, a radio frequency transmitter, a laser, or an RTP process. Other energy systems that quickly heat the getter material 90 to its activation temperature without adversely affecting the substrates may also be used. By focusing the high-intensity energy 95 only onto the getter material 90, the temperature of the getter material 90 rises much faster than that of the substrates 15 and 55. Moreover, since the materials from which the substrates 15 and 55 are made are reasonably resistant to heat transfer, only the small

interior regions 17 and 57 of the substrates adjacent to the getter material 90 generally reach the annealing temperatures of the substrates.

The large FED 100 has several advantages over conventional FEDs. One advantage is that the present invention allows more getter material 90 to be incorporated into the FED 100 in thinner layers. Referring to FIG. 2, in which like reference numbers refer to like parts in FIG. 1, a conventional FED is shown in which the getter material 90 is deposited onto a metal plate 80. The metal plate 80 is attached to either the faceplate 10 or the baseplate 50, and it is approximately 75  $\mu\text{m}$  thick. The getter material 90 in conventional FEDs is also approximately 75  $\mu\text{m}$  thick.

The present invention, however, eliminates the metal plate 80 which reduces the space required to incorporate the getter material into the FED. Moreover, by eliminating the metal plate 80, more getter material may be incorporated into an FED of the invention in less space compared to conventional FEDs. Referring again to FIG. 1, a 60  $\mu\text{m}$  layer of getter material 90a may be juxtaposed to a 50  $\mu\text{m}$  layer of getter material 90b; thus, for example, 110  $\mu\text{m}$  of getter material may be incorporated in an FED of the present invention in 40  $\mu\text{m}$  less space than 75  $\mu\text{m}$  of getter material in a conventional FED with a 75  $\mu\text{m}$  thick metal plate.

FIG. 3, which also uses like reference numbers to indicate like parts in FIG. 1, illustrates another embodiment of the invention in which the getter material 90 is deposited on various surfaces in a small FED 200. The small FED 200 has a faceplate 10, a baseplate 50, and a backplate 60. The backplate 60 is attached to the faceplate 10 such that it encloses the baseplate 50 in a vacuum space 42. A number of connectors 70 extend between the inner surface 11 of the faceplate 10 and the second electrically conductive layer 53 of the baseplate 50. The connectors 70 are bonded to the leads of the electrical conductive layer 53 in the baseplate 50 by a conductive bonding compound 72. The baseplate 50 is further supported by a support 14 positioned between the backplate 60 and the second surface 52 of the baseplate 50.

In the small display 200, a layer of getter material 90 may be deposited in its unactivated state on an interior surface 61 of the backplate 60, the inner surface 11 of the faceplate 10, or the second surface 52 of the baseplate 50. The getter material 90 in the small FED 200 is deposited and activated in the same manner as described above with respect to the large FED 100 in FIG. 1. Accordingly, only the small interior regions 17, 57 and 67 adjacent to the getter material 90 generally reach their respective annealing temperatures.

The small FED 200 also has several advantages over conventional FEDs. Referring to FIG. 4, in which like reference numbers indicate like parts in FIG. 3, a conventional small FED is depicted with a getter material 90 deposited on a metal plate 80. Typically, the metal plate 80 has a hole in the middle through which the conical support 14 is positioned. The metal plate 80, therefore, not only requires additional space to incorporate the getter material into the FED, but it is also subject to being dislodged from the support 14 and jostled within the vacuum space 42. As discussed above, the getter material may break away from the metal plate 80 and move throughout the vacuum space 42 until it causes shorting to occur between the emitters 54 and the conductive material 20. The FED 200 of the present invention substantially reduces the risk of particles coming loose and floating in the vacuum space 42 by securely attaching the getter material to the faceplate 10, baseplate 50, or backplate 60. The small FED 200 also allows more getter material 90 to be incorporated into the display for the reasons discussed above with respect to the large FED 100 in FIG. 1.

It will be appreciated that, although specific embodiments of the invention have been described herein for purposes of illustration, various modifications may be made without departing from the spirit and scope of the invention. Accordingly, the invention is not limited except as by the appended claims.

What is claimed is:

1. A method of applying a non-evaporable getter material to a substrate in a field emission display having a vacuum chamber a faceplate, and a baseplate wherein the substrate is a glass or a semiconductive component of one of the faceplate and the baseplate, the method comprising:

depositing unactivated getter material onto the substrate; after the getter material has been deposited on the substrate, selectively heating the getter material in a vacuum with an energy source focused substantially on the getter material, the heating being sufficient to raise the temperature of the getter material to its activation temperature; and

applying a thin film of binding metal onto the substrate prior to the depositing step.

2. The method of claim 1 wherein the applying step comprises sputtering a 1  $\mu\text{m}$ –20  $\mu\text{m}$  thick film of bonding metal on the substrate.

3. The method of claim 1 wherein the applying step comprises screen printing a 5  $\mu\text{m}$ –50  $\mu\text{m}$  thick film of bonding metal on the substrate.

4. A method of applying a non-evaporable getter material to a substrate in a field emission display having a vacuum chamber, a faceplate, and a baseplate, wherein the substrate is a glass or a semiconductive component of one of the faceplate and the baseplate, the method comprising:

depositing unactivated getter material onto the substrate by electroplating the getter material to the substrate; and

after the getter material has been deposited on the substrate, selectively heating the getter material in a vacuum with an energy source focused substantially on the getter material, the heating being sufficient to raise the temperature of the getter material to its activation temperature.

5. A method of applying a non-evaporable getter material to a substrate in a field emission display having a vacuum chamber, a faceplate and a baseplate, wherein the substrate is a glass or a semiconductive component of one of the faceplate and the baseplate, the method comprising:

depositing unactivated getter material onto the substrate by screen printing the getter material to the substrate; and

after the getter material has been deposited on the substrate, selectively heating the getter material in a vacuum with an energy source focused substantially on the getter material, the heating being sufficient to raise the temperature of the getter material to its activation temperature.

6. A method of applying a non-evaporable getter material to a substrate in a field emission display having a vacuum chamber, a faceplate, and a baseplate, wherein the substrate is a glass or a semiconductive component of one of the faceplate and the baseplate, the method comprising:

depositing unactivated getter material onto the substrate by electrophoresis deposition of the getter material to the substrate; and

after the getter material has been deposited on the substrate, selectively heating the getter material in a vacuum with an energy source focused substantially on

the getter material, the heating being sufficient to raise the temperature of the getter material to its activation temperature.

7. A method of applying a non-evaporable getter material to a substrate in a field emission display having a vacuum chamber, a faceplate, and a baseplate, wherein the substrate is a glass or a semiconductive component of one of the faceplate and the baseplate, the method comprising:

depositing unactivated getter material onto the substrate; and

after the getter material has been deposited on the substrate, selectively heating the getter material to its activation temperature with a microwave emitter.

8. The method of claim 1 wherein the activating step comprises selectively heating the getter material to its activation temperature with a laser.

9. The method of claim 1 wherein the activating step comprises selectively heating the getter material to its activation temperature with a radio frequency inductive coupling.

10. A method of manufacturing a flat panel display, comprising:

fabricating a baseplate by forming a plurality of emitters to project away from a baseplate substrate and by forming an extraction grid to have a plurality of openings aligned with the emitters;

constructing a faceplate by covering an inner surface of an optically transmissive faceplate substrate with an optically transmissive anode and covering the anode with a cathodoluminescent material;

installing an unactivated metallic getter material on at least one of the baseplate substrate and the faceplate substrate;

activating the getter material by selectively heating the getter material to an activation temperature by directing a discrete energy source to the getter material after the getter material is installed on at least one of the baseplate substrate and the faceplate substrate; and

applying a thin film of bonding material directly onto at least one of the baseplate substrate and the faceplate substrate prior to installing the getter material, and wherein installing the getter material comprises depositing the getter material on the bonding material.

11. The method of claim 10 wherein applying a thin film of bonding material comprises sputtering a 1  $\mu\text{m}$ –20  $\mu\text{m}$  thick film of bonding metal onto at least one of the baseplate substrate and the faceplate substrate.

12. The method of claim 10 wherein applying a thin film of bonding material comprises screen printing a 5  $\mu\text{m}$ –50  $\mu\text{m}$  thick film of bonding material onto at least one of the baseplate substrate and the faceplate substrate.

13. The method of claim 10 wherein installing the getter material comprises depositing a non-evaporable getter material directly onto at least one of the baseplate substrate and the faceplate substrate.

14. The method of claim 10 wherein activating the getter material comprises selectively heating the getter material to an activation temperature with a laser.

15. The method of claim 10 wherein activating the getter material comprises selectively heating the getter material to an activation temperature with a radio frequency inductive coupling.

16. A method of manufacturing a flat panel display, comprising:

fabricating a baseplate by forming a plurality of emitters to project away from a baseplate substrate and by

forming an extraction grid to have a plurality of openings aligned with the emitters;

constructing a faceplate by covering an inner surface of an optically transmissive faceplate substrate with an optically transmissive anode and covering the anode with a cathodoluminescent material;

installing an unactivated metallic getter material on at least one of the baseplate substrate and the faceplate substrate by screen printing a non-evaporable getter material directly onto at least one of the baseplate substrate and the faceplate substrate; and

activating the getter material by selectively heating the getter material to an activation temperature by directing a discrete energy source to the getter material after the getter material is installed on at least one of the baseplate substrate and the faceplate substrate.

17. A method of manufacturing a flat panel display, comprising:

fabricating a baseplate by forming a plurality of emitters to project away from a baseplate substrate and by forming an extraction grid to have a plurality of openings aligned with the emitters;

constructing a faceplate by covering an inner surface of an optically transmissive faceplate substrate with an optically transmissive anode and covering the anode with a cathodoluminescent material;

installing an unactivated metallic getter material on at least one of the baseplate substrate and the faceplate substrate by electrophoresis deposition of a nonevaporable getter material directly onto at least one of the baseplate substrate and the faceplate substrate; and

activating the getter material by selectively heating the getter material to an activation temperature by directing a discrete energy source to the getter material after the getter material is installed on at least one of the baseplate substrate and the faceplate substrate.

18. A method of manufacturing a flat panel display, comprising:

fabricating a baseplate by forming a plurality of emitters to project away from a baseplate substrate and by forming an extraction grid to have a plurality of openings aligned with the emitters;

constructing a faceplate by covering an inner surface of an optically transmissive faceplate substrate with an optically transmissive anode and covering the anode with a cathodoluminescent material;

installing an unactivated metallic getter material on at least one of the baseplate substrate and the faceplate substrate; and

activating the getter material by selectively heating the getter material to an activation temperature with a microwave emitter after the getter material is installed on at least one of the baseplate substrate and the faceplate substrate.

19. A method of manufacturing a baseplate for a field emission display, comprising:

forming a plurality of emitters over a baseplate substrate; fabricating an extraction grid to have a plurality of openings aligned with the emitters;

installing an unactivated non-evaporable metallic getter material directly on the baseplate substrate;

activating the getter material by selectively heating the getter material after the getter material is installed on the baseplate substrate; and

applying a thin film of bonding material directly onto the baseplate substrate prior to installing the getter material, and wherein installing the getter material comprises depositing the getter material on the bonding material.

20. The method of claim 19 wherein activating the getter material comprises selectively heating the getter material to an activation temperature with a laser.

21. The method of claim 19 wherein activating the getter material comprises selectively heating the getter material to an activation temperature with a radio frequency inductive coupling.

22. A method of manufacturing a baseplate for a field emission display, comprising:

forming a plurality of emitters over a baseplate substrate; fabricating an extraction grid to have a plurality of openings aligned with the emitters;

installing an unactivated non-evaporable metallic getter material directly on the baseplate substrate by electroplating the getter material directly onto the baseplate substrate; and

activating the getter material by selectively heating the getter material after the getter material is installed on the baseplate substrate.

23. A method of manufacturing a baseplate for a field emission display, comprising:

forming a plurality of emitters over a baseplate substrate; fabricating an extraction grid to have a plurality of openings aligned with the emitters;

installing an unactivated non-evaporable metallic getter material directly on the baseplate substrate by screen printing the getter material directly onto the baseplate substrate; and

activating the getter material by selectively heating the getter material after the getter material is installed on the baseplate substrate.

24. A method of manufacturing a baseplate for a field emission display comprising:

forming a plurality of emitters over a baseplate substrate; fabricating an extraction grid to have a plurality of openings aligned with the emitters;

installing an unactivated non-evaporable metallic getter material directly on the baseplate substrate by electrophoresis deposition of the getter material directly onto the baseplate substrate; and

activating the getter material by selectively heating the getter material after the getter material is installed on the baseplate substrate.

25. A method of manufacturing a baseplate for a field emission display, comprising:

forming a plurality of emitters over a baseplate substrate; fabricating an extraction grid to have a plurality of openings aligned with the emitters;

installing an unactivated non-evaporable metallic getter material directly on the baseplate substrate; and

activating the getter material by selectively heating the getter material to an activation temperature with a microwave emitter.

26. A method of manufacturing a faceplate for a field emission display comprising:

covering an optically transmissive faceplate substrate with an optically transmissive conductive film to form an anode;

disposing a cathodoluminescent material over the anode;

installing an unactivated non-evaporable metallic getter material directly on the faceplate substrate;

activating the getter material by selectively heating the getter material after the getter material is installed on the faceplate substrate; and

applying a thin film of bonding material directly onto the faceplate substrate prior to installing the getter material, and wherein installing the getter material comprises depositing the getter material on the bonding material.

27. The method of claim 26 wherein activating the getter material comprises selectively heating the getter material to an activation temperature with a laser.

28. The method of claim 26 wherein activating the getter material comprises selectively heating the getter material to an activation temperature with a radio frequency inductive coupling.

29. A method of manufacturing a faceplate for a field emission display comprising:

covering an optically transmissive faceplate substrate with an optically transmissive conductive film to form an anode;

disposing a cathodoluminescent material over the anode;

installing an unactivated non-evaporable metallic getter material directly on the faceplate substrate by electroplating the getter material directly onto the faceplate substrate; and

activating the getter material by selectively heating the getter material after the getter material is installed on the faceplate substrate.

30. A method of manufacturing a faceplate for a field emission display, comprising:

covering an optically transmissive faceplate substrate with an optically transmissive conductive film to form an anode;

disposing a cathodoluminescent material over the anode;

installing an unactivated non-evaporable metallic getter material directly on the faceplate substrate by screen printing the getter material directly onto the faceplate substrate; and

activating the getter material by selectively heating the getter material after the getter material is installed on the faceplate substrate.

31. A method of manufacturing a faceplate for a field emission display, comprising:

covering an optically transmissive faceplate substrate with an optically transmissive conductive film to form an anode;

disposing a cathodoluminescent material over the anode; installing an unactivated non-evaporable metallic getter material directly on the faceplate substrate by electrophoresis deposition of the getter material directly onto the faceplate substrate; and

activating the getter material by selectively heating the getter material after the getter material is installed on the faceplate substrate.

32. A method of manufacturing a faceplate for a field emission display, comprising:

covering an optically transmissive faceplate substrate with an optically transmissive conductive film to form an anode;

disposing a cathodoluminescent material over the anode; installing an unactivated non-evaporable metallic getter material directly on the faceplate substrate; and

## 11

activating the getter material by selectively heating the getter material to an activation temperature with a microwave emitter after the getter material is installed on the faceplate substrate.

**33.** A method of manufacturing a flat panel display comprising:

1 fabricating a first plate assembly to emit an energy the first plate assembly having a first substrate;

constructing an optically transmissive second plate assembly to receive the energy from the first plate assembly and to transmit light corresponding to the energy emitted from the first plate, the second plate assembly having a second substrate that is optically transmissive;

15 installing an unactivated non-evaporable metallic getter material on at least one of the first substrate and the second substrate;

activating the getter material by selectively heating the getter material after the getter material is installed on at least one of the first substrate and the second substrate; and

20 applying a thin film of bonding material directly onto at least one of the first substrate and the second substrate prior to installing the getter material, and wherein installing the getter material comprises depositing the getter material on the bonding material.

**34.** The method of claim 33 wherein activating the getter material comprises selectively heating the getter material to an activation temperature with a laser.

**35.** The method of claim 33 wherein activating the getter material comprises selectively heating the getter material to an activation temperature with a radio frequency inductive coupling.

**36.** A method of manufacturing a flat panel display comprising:

15 fabricating a first plate assembly to emit an energy the first plate assembly having a first substrate;

constructing an optically transmissive second plate assembly to receive the energy from the first plate assembly and to transmit light corresponding to the energy emitted from the first plate, the second plate assembly having a second substrate that is optically transmissive;

40 installing an unactivated non-evaporable metallic getter material on at least one of the first substrate and the second substrate by electroplating the getter material directly onto at least one of the first substrate and the second substrate; and

45 activating the getter material by selectively heating the getter material after the getter material is installed on at least one of the first substrate and the second substrate.

**37.** A method of manufacturing a flat panel display, comprising:

**12** fabricating a first plate assembly to emit an energy, the first plate assembly having a first substrate; constructing an optically transmissive second plate assembly to receive the energy from the first plate assembly and to transmit light corresponding to the energy emitted from the first plate, the second plate assembly having a second substrate that is optically transmissive;

installing an unactivated non-evaporable metallic getter material on at least one of the first substrate and the second substrate by screen printing the getter material directly onto at least one of the first substrate and the second substrate; and

activating the getter material by selectively heating the getter material after the getter material is installed on at least one of the first substrate and the second substrate.

**38.** A method of manufacturing a flat panel display, comprising:

fabricating a first plate assembly to emit an energy, the first plate assembly having a first substrate;

constructing an optically transmissive second plate assembly to receive the energy from the first plate assembly and to transmit light corresponding to the energy emitted from the first plate, the second plate assembly having a second substrate that is optically transmissive;

installing an unactivated non-evaporable metallic getter material on at least one of the first substrate and the second substrate by electrophoresis deposition of the getter material directly onto at least one of the first substrate and the second substrate; and

activating the getter material by selectively heating the getter material after the getter material is installed on at least one of the first substrate and the second substrate.

**39.** A method of manufacturing a flat panel display, comprising:

fabricating a first plate assembly to emit an energy, the first plate assembly having a first substrate;

constructing an optically transmissive second plate assembly to receive the energy from the first plate assembly and to transmit light corresponding to the energy emitted from the first plate, the second plate assembly having a second substrate that is optically transmissive;

installing an unactivated non-evaporable metallic getter material on at least one of the first substrate and the second substrate; and

activating the getter material by selectively heating the getter material to an activation temperature with a microwave emitter after the getter material is installed on at least one of the first substrate and the second substrate.

\* \* \* \* \*

UNITED STATES PATENT AND TRADEMARK OFFICE  
**CERTIFICATE OF CORRECTION**

PATENT NO. : 6,033,278

DATED : March 7, 2000

INVENTOR(S) : Charles M. Watkins et al.

It is certified that error appears in the above-identified patent and that said Letters Patent is hereby corrected as shown below:

On the title page,  
[75] Inventors

Reads

Should Read

Watkins; Cathey

“Iowa”

--Idaho--

Column, Line

Reads

Should Read

Column 6, Line 10

“chamber a faceplate”

-- chamber, a faceplate --

Column 6, Line 10

“baseplate wherein”

-- baseplate, wherin --

Column 6, Line 44

“faceplace and a”

-- faceplate, and a --

Column 8, Line 30

“nonevaporable”

-- non-evaporable --

Column 8, Line 40

“forming,”

-- forming --

Column 9, Line 37

“setter”

-- getter --

Column 9, Line 39

“display comprising”

-- display, comprising --

Column 9, Line 62

“display comprising”

-- display, comprising --

Column 10, Line 19

“display comprising”

-- display, comprising --

Signed and Sealed this

First Day of May, 2001

Attest:



NICHOLAS P. GODICI

Attesting Officer

Acting Director of the United States Patent and Trademark Office